

1

2,732,316

## HARDENING OF GELATIN

George July, Edward Bowes Knott, and Felix Pollak, Wealdstone, Harrow, England, assignors to Eastman Kodak Company, Rochester, N. Y., a corporation of New Jersey

No Drawing. Application December 3, 1952,  
Serial No. 323,924

7 Claims. (Cl. 117—62)

This invention relates to the hardening of gelatin particularly in photographic emulsions with 1:3-dihydroxymethylbenzimidazol-2-ones.

In the case of gelatin which is to be treated with aqueous solutions, as exemplified by photographic emulsions which are treated with processing solutions, it is particularly desirable that the gelatin have properties whereby it is resistant to the effects of the aqueous solution. It is a particular advantage if the gelatin material is not only resistant to water at normal temperature but to water at elevated temperatures because in the case of photographic emulsions resistance to hot water would permit the hot processing of the gelatin emulsion thus shortening the time for the processing operations.

One object of our invention is to provide a gelatin which is resistant to the effect of water at elevated temperature. Another object of our invention is to provide gelatin photographic emulsions which may be hot processed without break down of the physical structure thereof. A further object of our invention is to provide compositions of gelatin in which a small amount of a 1:3-dihydroxymethylbenzimidazol-2-one is present therein. Other objects of our invention will appear herein.

We have found that when gelatin is treated with a 1:3-dihydroxymethylbenzimidazol-2-one, or any gelatin layers or photographic gelatin emulsion layers are treated with a 1:3-dihydroxymethylbenzimidazol-2-one, the resulting product is resistant to the effect of hot water or of hot aqueous processing solutions and that in the case of photographic emulsions so treated higher speed and gamma are obtained than with emulsions not so treated and having equal fog characteristics or where equal development times are used higher speed and gamma and lower fog characteristics are obtained than for emulsions not so treated. We have found that gelatin hardened in accordance with our invention is useful either in color photography or in black-and-white photography.

The hardeners which are employed in accordance with our invention have the structural formula:



where R is either hydrogen, alkyl or a halogen substituent. Compounds of this type may be prepared as illustrated by the following examples.

### Example 1

30 parts of benzimidazol-2-one in 200 parts of water was slowly warmed with 75 parts of 40% formalin until the solid just dissolved in the liquid portion thereof. The small amount of residual black matter was filtered off and the solution was cooled to 0° C. Sandy crystals formed which were separated from the liquid and recrystallized from hot water. 54.22 parts of 1:3-di(hydroxymethyl)-benzimidazol-2-one was obtained melting at 163—164° C.

2

### Example 2

2 parts of 5-methylbenzimidazol-2-one was mixed with 10 parts of water and 5 parts of 40% formalin and the mixture was slowly warmed so as to dissolve the solid material therein. The solution thus formed was filtered and cooled to 0° C. which resulted in the formation of pale orange, sandy crystals. These crystals were separated from the liquid and recrystallized from hot water. 2 parts of 1:3-di(hydroxymethyl)-5-methyl-benzimidazol-2-one melting at 176—178° C. was obtained.

In the carrying out of our invention the gelatin may be hardened either by incorporating hardener directly in the gelatin, or layers of gelatin which have been coated out onto a support may be treated with a solution of the hardener so as to impart a hardening effect thereto. The hardening action on the gelatin in accordance with our invention takes place to the best effect at a pH value of at least 8. Although the hardener in accordance with our invention modifies the properties of the gelatin when employed therewith in any proportion, we have found that amounts of the hardener within the range of .1—10% based on the weight of the gelatin are the most desirable in carrying out the hardening of gelatin in accordance with our invention. In the compounds employed for hardening in accordance with our invention the benzene ring therein may either be unsubstituted except for the imidazole ring thereon or an alkyl or halogen substituent may be present on the benzene ring. If an alkyl group is the substituent on the ring it is desirable that it be selected from those alkyls which have 1—4 carbon atoms such as methyl, ethyl, isopropyl or the like. If a halogen substituent is employed this substituent is most desirably chlorine although the hardening action on the gelatin treated therewith will be effective if some other halogen substituent such as bromine or fluorine is used.

The following examples illustrate the hardening of gelatin in accordance with our invention:

### Example 3

40 A strip of photographic film having three layers of a gelatin emulsion thereon each sensitive to a different color such as is employed in color photography was immersed for 4 minutes at 100° F. in a solution consisting of 1 gram of 1:3-dihydroxymethylbenzimidazol-2-one, 15 grams of sodium sulfate, 100 cc. of water and a sodium borate-boric acid buffer to maintain the solution at a pH of 9. After immersing the film strip for the specified time it was rinsed in water at 100° F. for two minutes and then developed at 100° F. The film strip was subjected to washing with 50 water having a temperature of 160° F. and no change occurred in the emulsion layer.

### Example 4

55 The procedure of Example 3 was repeated except that the hardening solution was maintained at a pH of 8 and the film was dried first and then subjected to photographic processing. The resulting film strip was subjected to a washing with water having a temperature of 160° F. and no change was found to occur in the emulsion layer.

### Example 5

60 The procedure of Example 4 was repeated but with the addition that after drying the film it was immersed in a solution in water of resorcinol (1/4%) and resorcylic aldehyde (1/4%). A very hard film was obtained. In proceeding according to the above examples it was found that when the layers were processed according to Examples 4 and 5 that the resulting emulsion layers had similar photographic properties and a high photographic density was obtained thereby. It was also noted in these examples that the speed of the yellow layer was not as

great as in the case of those emulsions which had not been subjected to such hardening. However, this lowering of speed could readily be compensated for by increasing the first development time. In many cases the speed reduction of the yellow layer is of advantage such as in those color processes which suffer from a too rapid development of the yellow layer. The hardening of the emulsion layer as described in Example 3 gave good results and was fully equivalent to that obtained with formalin hardening but with the additional advantage, however, that in the case of the formalin hardening a washing in water after treatment with the formalin produced a high fog in the yellow layer, whereas in the case of the film strip hardened in accordance with our invention no such fogging resulted. The following table compares the product hardened in accordance with our invention and that hardened with formalin.

| Hardening time             | Test Solution |        | Control (formalin) |         |
|----------------------------|---------------|--------|--------------------|---------|
|                            | 1 min.        | 4 min. | 20 sec.            | 40 sec. |
| Development time..... min. | 4             | 4      | 4                  | 4       |
| Fog.....                   | 0.21          | 0.21   | 0.26               | 0.27    |
| Speed.....                 | 2.35          | 2.20   | 2.18               | 2.09    |
| Gamma.....                 | 1.03          | 0.95   | 0.80               | 0.74    |
| Development time..... min. | 8             | 8      | 8                  | 8       |
| Fog.....                   | 0.31          | 0.42   | 0.50               | 0.66    |
| Speed.....                 | 2.35          | 2.26   | 2.16               | 1.96    |
| Gamma.....                 | 1.64          | 1.26   | 1.17               | 1.00    |

Thus it may be seen that for equal development times the emulsion hardened in accordance with our invention exhibited higher speed and gamma and lower fog than in the case of the formalin hardened emulsion.

We have also found that the hardeners referred to above are effective for hardening gelatin when incorporated in compositions thereof as illustrated by the following examples:

#### Example 6

Three samples of a gelatin-silver halide negative emulsion were taken and in two of those samples hardeners in accordance with our invention were incorporated. The melting point of the emulsion was increased by those additions as shown by the following:

90° F. melting point of untreated emulsion.

146° F. melting point of the emulsion to which has been added 1/4 gram of 1:3-di(hydroxymethyl)-benzimidazol-2-one per liter of emulsion.

207° F. melting point of emulsion containing 1 gram of 1:3-di(hydroxymethyl)-benzimidazol-2-one per liter of emulsion.

Upon coating out of the emulsion and subjecting the same to incubation the hardening thereof is still further increased.

#### Example 7

A fast negative chlorobromide gelatin emulsion was taken and one sample was untreated and two samples were mixed with hardener in accordance with our invention. The results obtained were as follows:

|                                                                                                                      | Initial,<br>°F. | After Incubation,<br>°F. |
|----------------------------------------------------------------------------------------------------------------------|-----------------|--------------------------|
| Melting point of untreated emulsion                                                                                  | 91              | 92                       |
| Melting point of emulsion containing 1/4 gram of 1:3-di(hydroxymethyl)-benzimidazol-2-one per liter of emulsion..... | 102             | 200                      |
| Melting point of emulsion containing 1 gram of 1:3-di(hydroxymethyl)-benzimidazol-2-one per liter.....               | 105             | 207                      |

#### Example 8

16 mm. film having thereon a highly sensitive emul-

sion was immersed in a solution for two minutes having the following composition:

0.3 part of 1:3-di(hydroxymethyl)-5-methylbenzimidazol-2-one

5 15 parts of Na<sub>2</sub>SO<sub>4</sub>

2 parts of Na<sub>2</sub>CO<sub>3</sub>·H<sub>2</sub>O

Water to make 100 parts.

The film after hardening in this solution at 100° F. for two minutes was washed with water for one minute and then processed in a hydroquinone-metol type developer for 4, 8 and 16 minutes. The film after processing was examined and was found to be well hardened for each of the various development times which were used. This hardening compound was also employed to treat photographic film of the color type having three layers of different color sensitivities thereon. It was found that the resulting product had excellent hardness and fog was kept to a minimum.

We claim:

1. A composition of gelatin and a compound having the structural formula



R being a substituent selected from the group consisting of hydrogen, lower alkyl, chlorine, bromine and fluorine.

2. A composition of gelatin and 1:3-dihydroxymethylbenzimidazol-2-one.

3. A composition of gelatin and 1:3-dihydroxymethyl-5-methylbenzimidazol-2-one.

35 4. A method of hardening a gelatin layer which comprises immersing the layer in an aqueous solution of a compound having the structural formula



R being a substituent selected from the group consisting of hydrogen, lower alkyl, chlorine, bromine and fluorine.

45 5. A method of hardening a gelatin layer which comprises immersing the layer in an aqueous solution of 1:3-dihydroxymethylbenzimidazol-2-one.

50 6. A method of hardening a gelatin layer which comprises incorporating in an aqueous gelatin composition a small proportion of a compound having the structural formula:



R being a substituent selected from the group consisting of hydrogen, lower alkyl, chlorine, bromine and fluorine, and subsequently coating out the composition onto a support.

60 7. A method of hardening a gelatin layer which comprises incorporating in an aqueous gelatin composition a small proportion of 1:3-dihydroxymethylbenzimidazol-2-one and coating out the resulting composition onto a support therefor.

#### References Cited in the file of this patent

#### UNITED STATES PATENTS

- 2,333,329 Miglarese Nov. 2, 1943  
 2,341,877 Middleton et al. Feb. 15, 1944  
 2,347,644 Sell May 2, 1944  
 2,572,988 Collins et al. Oct. 30, 1951